

# UNITED STATES PATENT OFFICE.

HERBERT ABRAHAM, OF BOUND BROOK, NEW JERSEY, AND HAROLD W. HAINES, OF NEW YORK, N. Y., ASSIGNEES TO IMPERVIOUS PRODUCTS COMPANY, A CORPORATION OF NEW YORK.

## CEMENT-MAKING.

1,134,573.

Specification of Letters Patent.

Patented Apr. 6, 1915.

No Drawing.

Application filed March 9, 1910. Serial No. 548,114.

To all whom it may concern:

Be it known that we, HERBERT ABRAHAM and HAROLD W. HAINES, citizens of the United States, the former a resident of 5 Boundbrook, county of Somerset, and State of New Jersey, and the latter a resident of the borough of Manhattan, New York city, New York, have jointly invented certain new and useful Improvements in Cement-making, of which the following is a specification.

Our invention relates to the production of water-proof hydraulic cement, and to the production of miscible pastes for use in the 15 gaging water employed in the preparation of said waterproof materials, and to the accomplishment of these results preferably without impairing the strength of the finished cement.

Many attempts have been made to render 20 hydraulic cement waterproof, but as far as we are aware, none of these have proven satisfactory. In some cases a very limited degree of water-tightness has been secured, but 25 generally at the expense of the strength of the finished product, and this decrease in strength has often unfitted such product for commercial use. Thus the addition of fatty bodies or soaps, whether soluble or in- 30 soluble, greatly decreases the strength of the hydraulic cement, if used in more than insignificant amounts, while adding greatly to the cost. Even when added in small quantities they notably affect the strength 35 without imparting any marked waterproofing effects.

By means of our invention we have entirely overcome all of these objections, have succeeded in obtaining a satisfactory hydraulic cement, mortar or concrete that is 40 substantially waterproof or water-tight at a very moderate cost, and which will not deteriorate or decrease in efficiency during service. We have accomplished this in our 45 preferred method, not only without materially diminishing the strength of the finished structure, but in fact in most cases have been able to increase its strength, especially with lean mixtures.

We will now proceed to describe the preferred embodiment of our improved process 50 and product.

In carrying out our improved process, we

mix a suitable carrier, preferably a more or less insoluble inorganic hydroxid, capable of forming with water a viscous plastic mixture, such as slaked lime, in the form of a paste, with a suitable proportion of a viscous unsaponifiable bituminous liquid which must be so chosen that it will not materially lessen the strength of the finished cement. Certain liquid asphaltums or asphaltum oils have been found suitable, and indeed some of them materially increase the strength of the finished cement. The bituminous liquid is preferably added in small quantities at a time and the mixture triturated or ground during such additions to intimately mix the ingredients together. We then add water to the resulting mixture, preferably in small quantities at a time, and preferably continue the said trituration or grinding until a suitable proportion of water has been incorporated to render the paste miscible with water without 75 liberation of the bituminous liquid. We thus produce a miscible paste suitable for use in the gaging water ordinarily employed in preparing hydraulic cement, mortar and concrete, which paste is miscible with either 80 cold or hot water in any proportions without liberation of the bituminous liquid even on long standing. This miscible paste is then mixed with the gaging water and the resulting liquid incorporated with the hydraulic cement, mortar or concrete in the ordinary manner.

During the process of setting, the inorganic hydroxid which we preferably employ as the carrier for the bituminous matter, reacts 90 chemically, thereby increasing the strength of the resultant product. In this re-action, the inorganic hydroxid, being a basic body, may combine chemically with the acidic constituents present, such as silica 95 or else it may act with the carbon dioxide absorbed from the atmosphere to form carbonate. The bituminous liquid does not undergo any chemical change during the process of setting, but is retained mechanically 100 in the pores of the structure of the cement, mortar or concrete, or of the structure composed of the chemically combined hydroxid and cement, mortar or concrete, without exuding or leaching out with the surplus water 105 as the product sets and dries. The result-

ant product is waterproof and has in most cases greater strength than would be possessed without such treatment.

While it will, of course, be understood that numerous changes in or departures from the specific ingredients, proportions and steps of our process hereinafter described may be made, we will now proceed to describe the best form known to us for carrying out our improved process and the best ingredients and proportions for use therein.

Although according to our invention any suitable more or less insoluble inorganic substance, capable of forming with water a viscous plastic mixture, may be employed as carrier, we prefer to use a hydroxid for the reasons herein mentioned, and particularly slaked lime on account of its abundance and cheapness. Preferably the lime should be pure. We have found that limes known commercially as "fat" limes or "finishing" limes are best suited to our purpose, for they will not result in the formation of coarse-grained gray pastes which are liable to permit the asphaltum to separate on dilution, as is the case with the impurer varieties. We are likewise influenced in selecting pure limes, by the fact that the magnesia existing in the impurer varieties hydrates with difficulty, and the presence of anhydrous magnesia is generally recognized to exert a deleterious action on cements. We hydrate unslaked lime forming a paste containing preferably an equivalent of one part by weight of the anhydrous lime (calcium oxid) to one and a half parts by weight of water. We then mix two and a half parts by weight of this paste with preferably two parts by weight of a viscous, unsaponifiable bituminous liquid. This we preferably add in small quantities at a time to the lime paste, triturating or grinding the mixture in a suitable apparatus during such additions. Any suitable apparatus may be used for this purpose, as for example, the triturating machine ordinarily used in grinding putties, which is generally known as an "edge runner" or "chaser." The mechanical manipulation or trituration intimately mixes the ingredients together, and is preferably continued until the mass possesses a uniform color and a smooth texture. Water is then added, preferably in small quantities at a time, and preferably the grinding or trituration is continued, although any suitable method of mixing may be employed at this stage of the process. We prefer to add water to the paste until the resulting mixture attains a uniform smooth buttery consistency and becomes miscible with water in all proportions without causing any separation of the asphaltum oil. This miscible paste is now adapted for use with the gaging water ordinarily employed in making hy-

draulic cement, mortar and concrete. The resulting cement, when set, is thoroughly waterproof and possesses great strength. The actual waterproofing, however, is effected by the asphaltum, which is retained by capillarity in the pores of the finished structure. Although the asphaltum will in no way interfere with the evaporation of the excess water, yet it will effectually prevent the absorption of external moisture. It will be noted that the miscible paste itself loses the property of mixing with water, after it has once been allowed to dry in the air or otherwise.

In place of the calcium hydroxid or slaked lime, any other suitable more or less insoluble inorganic hydroxid capable of forming with water a viscous plastic mixture as, for example, iron hydroxid, aluminum hydroxid, etc., may be employed with more or less satisfactory results.

While any other suitable carrier may be employed, if desired, such as plastic clays or the like, and the benefits of our invention in some of its features may be realized to a greater or less extent, we prefer to use as a carrier one of the inorganic hydroxids, as they serve to increase the strength of the resulting product because of their chemical union with the aggregate, whereas the use of an inert inorganic substance, such as plastic clays, tends to decrease the strength.

We are aware that it is not new to introduce hydrated lime alone into cement mixtures, and that, when thus introduced, it increases the plasticity and ease of working of the mixture, and serves, to a limited extent, to reduce the porosity of the structure with which it is combined. It fails, however, to render the cement waterproof. As far as we know, it is entirely novel to employ lime or any equivalent inorganic hydroxid, or any more or less insoluble inorganic substance capable of forming with water a viscous plastic mixture, as a vehicle for carrying and introducing an unsaponifiable bituminous liquid, into the structure of cement, mortar or concrete. Attempts of this general nature have been made, but, as far as we are aware, have failed. For example, the use of solid bituminous matter with clay as the carrier, has been suggested. A satisfactory waterproofing effect, however, cannot be obtained from a solid bituminous substance as thus employed. The bituminous matter must be of the proper consistency, neither too stiff or solid, nor too thin or liquid, as set forth below.

When lime is used as the carrier or vehicle for introducing the asphaltum in our process, it imparts to the mixtures the characteristic plasticity and ease of working referred to above.

While we prefer to use, as our unsaponifiable bituminous liquid, liquid asphaltum

or asphaltum oil so-called, because of its abundance and cheapness, any other suitable unsaponifiable bituminous liquid of a proper consistency may be employed, such as bitumens, tars and pitches of a hydrocarbon nature, as for example, coal tar pitch, or the like. The bituminous substance best adapted for our purpose must at ordinary temperatures be neither too liquid nor too stiff. We have found that, if it is too thin or liquid, it is not apt to be effectively retained in the pores of the hydraulic cement and that it will, moreover, fail to give the best waterproofing qualities even if it be actually retained. On the other hand, if it is too stiff or solid, it will fail to distribute itself properly in the pores of the finished structure, and will in that case behave as an inert substance without imparting satisfactory waterproofing effects. We have found that under the latter circumstances the set cement is actually weakened. A viscous unsaponifiable bituminous liquid, such as asphaltum oil or coal tar pitch, gives the best results. It is sufficiently liquid both to unite intimately with the carrier and the water to form the miscible paste, and to distribute itself properly in the pores of the cement, mortar or concrete, and also sufficiently viscous not to exude or leach out during and after the process of setting. We have found, moreover, that viscous liquids of this description will not be displaced from the pores of the set cement, mortar or concrete, or permit water to permeate even when subjected to considerable hydro static pressure. When the liquid asphaltum is added to the calcium hydroxid, the latter should be in the form of a stiff paste. We have found that if the paste is too dry, the asphalt will inhibit the subsequent addition and incorporation of water; and that if too moist, the asphalt itself cannot properly be incorporated.

The process of titurating the lime paste with the liquid asphaltum, is carried on preferably in the cold. This trituration breaks up the lime and causes both the lime and the bituminous liquid to be intimately mixed and incorporated with each other in a very fine state of division. We have found that the mere stirring of the ingredients together is not as satisfactory as a trituration or grinding. A grinding action, such as is effected by the use of the above mentioned type of machine, gives the best results.

The addition of too much asphalt will render the paste incapable of being mixed with water. In practice, we have found that it is not advisable to incorporate more than two parts by weight of asphalt with the equivalent of one part by weight of the anhydrous lime. The capacity of different hydroxids for carrying the bituminous liquid varies greatly. Whereas in the case

of calcium hydroxid about two parts by weight of asphaltum oil may be incorporated with the equivalent of one part by weight of the anhydrous oxid, in the case of iron hydroxid about three parts by weight of asphaltum oil may be incorporated, and with aluminum hydroxid about five parts by weight. It is obviously desirable that the resulting paste should carry the maximum quantity of asphaltum and the minimum quantity of water consistent with easy and complete miscibility with the gaging water.

In using the paste the best results will generally be obtained when the volume of asphaltum oil introduced approaches the volume of voids contained in the mixture of cement and aggregate. The presence of too large a quantity of asphaltum tends to weaken the strength of the finished product. This will be the case when the volume of asphaltum exceeds the volume of pores or voids or interstices in the structure, for it will then tend to separate and prevent the contiguous particles from bonding properly. A decrease in the volume of asphaltum introduced usually decreases the waterproofing effect. This, however, may be compensated for by an increased thickness of the treated layer of cement, mortar or concrete, and we have found in practice that in this manner a very efficient waterproofing may be imparted by introducing a volume of asphaltum considerably less than the volume of voids.

The volume of voids will to a certain extent vary with the varying conditions of each case. Thus the total volume of the pores, interstices or voids in the finished product will vary, for example, with the different kinds of sand used. The finer the sand or the larger the amount used in the mixture, the greater will be the said volume of voids. In this latter case a relatively larger quantity of bituminous liquid would obviously be required than when for example, a coarser or graded variety of sand, or a richer mixture were employed. In general, the addition of 10% by weight of our miscible paste based on the combined weights of sand and cement gives satisfactory results. With concrete, the crushed stone or gravel should be disregarded in making this calculation, for these substances do not materially influence the total volume of voids.

Cement, mortar and concrete waterproofed as described will bond equally well with surfaces of an untreated material as with surfaces which have similarly been waterproofed, and the addition of our waterproofing paste does not interfere, as far as we have been able to ascertain, with the setting of the mixture. We prefer to use a bituminous liquid free from volatile ingredients, as it is less likely to be affected by

70

75

80

85

90

95

100

105

110

115

120

125

130

exposure to the elements. The presence of the bituminous liquid renders the cement structure more highly resistant to the action of the elements, for it prevents access of moisture and frost, and the formation of surface checks and expansion cracks. It likewise serves to preserve any steel that may be used for reinforcing purposes, and to protect it from rusting in the manner of bituminous paints, and without interfering with the bond between the metal and the cement, mortar or concrete.

In many instances it is desirable to impart to the cement structure a color other than that characteristic of ordinary cement. It is not new to mix certain inert mineral pigments with the ingredients of the aggregate to produce colored decorative effects. These pigments are usually added in small quantities, for it requires but a small amount of an intense pigment to modify the natural color of the mass. In our improved process this coloring may be advantageously effected by grinding a suitable percentage of the pigment with the ingredients of the miscible paste. The paste may, therefore, be advantageously used as a vehicle for conveying and distributing the pigment throughout the cement mixture. It will effect this more uniformly and with greater ease than would be the case if the pigment were incorporated with the aggregate in a dry state. The pigment may be mixed with the paste either before or after the asphaltum has been added, without apparently affecting its miscibility. The percentage of pigment used should be maintained as low as possible for it is an inert substance, and as such tends to weaken the structure. If the pigment exists in the form of a more or less insoluble inorganic substance capable of forming with water a viscous plastic mixture, it may obviously serve to replace the hydroxid either wholly or in part, as a carrier for the bituminous liquid. As an example, we have in some cases found it desirable to incorporate one part by weight of strong natural red oxide of iron with five parts by weight of the miscible paste. It will, of course, be understood that other inert mineral pigments, such as yellow ocher, lamp black, lime proof greens and the like, may be similarly employed in suitable amounts.

To avoid repetition, especially in the claims, we use the word "cement" in its more or less popular sense to include all hydraulic cement, mortar, concrete or artificial stone made with hydraulic cement.

By means of our improved process a very large proportion of bituminous matter to carrier may be incorporated into the cement, mortar or concrete. In most cases the proportion of bituminous matter will be in excess of that of the carrier, and where the preferred form of our improved process is

carried out, the proportion will be double or more than double that of the carrier, thus affording a very high degree of efficiency.

What we claim as new and desire to secure by Letters Patent, is:

1. The process of making a paste miscible with water, adapted for use with the gaging water used in preparing hydraulic cement or the like, which consists in mixing a substantially insoluble inorganic substance capable of forming with water a viscous plastic mixture, water, and a viscous unsaponifiable bituminous liquid which will not materially lessen the strength of the cement in suitable proportions. 70 75

2. The process of making a paste adapted for use with the gaging water used in preparing hydraulic cement, or the like, which consists in mixing a substantially insoluble inorganic substance capable of forming with water a viscous plastic mixture, and water in suitable proportions, and adding to the paste thus formed a suitable proportion of a viscous unsaponifiable bituminous liquid which will increase the strength of the cement, the mixture being triturated or ground until of a uniform color and smooth texture, and then adding water during the triturating or grinding until the resulting paste becomes miscible with water without 80 85 90 liberation of the bituminous liquid. 95

3. The process of making a paste adapted for use with the gaging water used in preparing hydraulic cement, or the like, which consists in mixing a paste of calcium hydroxid with a viscous unsaponifiable bituminous liquid which will not materially lessen the strength of the cement and water in suitable proportions so that the paste becomes miscible with water. 100 105

4. The process of making a paste adapted for use with the gaging water used in preparing hydraulic cement, or the like, which consists in mixing a paste of calcium hydroxid with a viscous unsaponifiable bituminous liquid which will increase the strength of the cement in suitable proportions, the said liquid being added in small quantities at a time, and the mixture being triturated or ground during such additions 110 until of a uniform color and smooth texture, and then adding water and mixing the resulting product until the paste becomes miscible with water without liberation of the bituminous liquid. 115 120

5. The process of making a paste adapted for use with gaging water in preparing hydraulic cement, or the like, which consists in intimately mixing a viscous unsaponifiable bituminous liquid which will not materially weaken the cement, a suitable carrier therefor and water, the amount of bituminous liquid thus mixed being in excess of the amount of the carrier. 125

6. The process of making a paste adapted 13

- for use with gaging water in preparing hydraulic cement or the like, which consists in mixing in suitable proportions, a viscous unsaponifiable bituminous liquid which will 5 not materially weaken the cement, a suitable carrier capable of forming with water a viscous plastic mixture, and water. 70
7. The process of making a paste adapted for use with gaging water in preparing hydraulic cement, or the like, which consists in mixing in suitable proportions, and in a suitable manner, a more or less insoluble inorganic substance capable of forming with water a viscous plastic mixture, a suitable 10 pigment, water, and a viscous unsaponifiable bituminous liquid which will increase the strength of the cement. 80
8. The process of preparing waterproof cement, or the like, which consists in inter- 20 nately mixing in suitable proportions, a substantially insoluble inorganic hydroxid capable of forming with water a viscous plastic mixture, water, and a viscous unsaponifiable bituminous liquid which will increase 25 the strength of the cement, mixing the paste thus formed with gaging water, and mixing the resulting liquid with cement constituents before setting. 90
9. The process of preparing waterproof 30 cement or the like, which consists in intimately mixing a viscous unsaponifiable bituminous liquid which will not materially lessen the strength of the cement and a suitable carrier therefor, and in combining 35 therewith water in a manner and in amounts until a miscible paste is formed from which the bituminous liquid will not be liberated when the paste is mixed with additional water, mixing such paste with gaging water, 40 and mixing the resulting liquid with other constituents of cement before setting. 95
10. A miscible paste for use with gaging water in preparing hydraulic cement, or the like, containing a substantially insoluble in- 45 organic substance capable of forming with water a viscous plastic mixture, a viscous unsaponifiable bituminous liquid which will not materially weaken the cement, and water in suitable proportions. 100
- 50 11. A miscible paste for use with gaging water in preparing hydraulic cement, and the like, containing two parts by weight or less of a viscous unsaponifiable bituminous liquid which will increase the strength 55 of the cement, the equivalent of one part by weight of anhydrous lime, and sufficient water to render the paste readily miscible. 110
12. A miscible paste for use with gaging water in preparing hydraulic cement, or the 60 like, containing liquid asphaltum of a character to increase the strength of the cement, slaked lime, and water, combined in suitable proportions and triturated or ground together. 115
- 65 13. A miscible paste used with gaging water in preparing hydraulic cement, or the like, containing intimately mixed together a viscous unsaponifiable bituminous liquid of a character not to materially lessen the strength of the cement, water, and a suitable 70 carrier therefor. 120
14. A miscible paste for use with gaging water in preparing hydraulic cement, or the like, containing a viscous unsaponifiable bi- 75 tuminous liquid of a character to materially increase the strength of the cement, a sub- stantially insoluble inorganic hydroxid ca- 80 pable of forming with water a viscous plas- tic mixture, and water, all mixed and com- bined in suitable proportions. 85
15. A miscible paste for use with gaging water in preparing hydraulic cement, or the like, containing intimately mixed together, a viscous unsaponifiable bituminous liquid which will not materially weaken the ce- 90 ment, a suitable colored pigment capable of forming with water a viscous plastic mix- ture, and water. 95
16. A colored miscible paste for use with gaging water in preparing hydraulic cement, 90 containing a viscous unsaponifiable bitumi- nous liquid which will increase the strength of the cement, a somewhat insoluble in- 95 organic substance capable of forming with water a viscous plastic mixture, a pigment, and water, all intimately mixed and com- bined in suitable proportions. 100
17. A hydraulic cement, treated to make it waterproof, containing therein, when set, a substantially insoluble inorganic substance 100 and a viscous unsaponifiable bituminous liquid which does not materially weaken the cement. 110
18. A hydraulic cement, treated to make it waterproof, containing in addition to ce- 105 ment constituents, inorganic derivatives of a substantially insoluble inorganic hydroxid, and also a viscous unsaponifiable bituminous liquid distributed in the pores of the result- ing product which increases the strength of the cement. 115
19. A hydraulic cement, treated to make it waterproof, containing inorganic derivatives of calcium hydroxid in excess of those nor- mally present in the untreated cement, when 115 set, and also a viscous unsaponifiable bitu- minous liquid distributed in the pores of the cement which does not materially decrease the strength of the cement. 120
20. A waterproof hydraulic cement, made 120 waterproof by the presence in its pores of a viscous unsaponifiable bituminous liquid of a character not to materially weaken the cement. 125
21. A waterproof hydraulic cement, made 125 waterproof by the presence in its pores of asphaltum oil of a character to increase the strength of the cement. 130
22. A waterproof hydraulic cement, con- 130 taining a finely divided suitable colored pig-

ment and a viscous unsaponifiable bituminous liquid distributed in the pores of the cement which does not materially weaken the cement.

- 5 23. A colored hydraulic cement, treated to make it waterproof, containing in addition to cement constituents, when set, a substantially insoluble inorganic substance, and a viscous unsaponifiable bituminous liquid of  
10 a character to increase the strength of the

cement, and a finely divided suitable pigment.

In testimony whereof, we have signed our names to this specification, in the presence of two subscribing witnesses.

HERBERT ABRAHAM.  
HAROLD W. HAINES.

Witnesses:

EDWIN SEGER,  
E. A. NIEDERHAUSER.